

## UNITED STATES PATENT OFFICE

2,155,046

## INHIBITED DETERGENT COMPOSITION

Carroll L. Griffith and Lloyd A. Hall, Chicago, Ill.,  
assignors to The Griffith Laboratories, Inc.,  
Chicago, Ill., a corporation of Illinois

No Drawing. Application February 29, 1936, Serial No. 66,436. Renewed March 8, 1939

10 Claims.

(Cl. 87—5)

The present invention relates to alkaline detergent materials for metal pieces, especially those having surfaces of tin, zinc, iron or aluminum, which is effective to clean the same without deleterious action such as corrosion, dissolution, "spangling" or checking.

The use of alkaline agents is well known for cleaning metal ware of zinc, aluminum or tin plate, such as milk cans, baking pans, etc., which have oil, grease or fat, burned-on flour, milk curds, etc. It is realized that baths of these agents are usually injurious to the metal in the concentrations and at the elevated temperatures and the time of action ordinarily employed. It is also known that inhibiting agents are added to minimize or prevent such deleterious action. Some of these inhibited detergent compounds are effective when the metal pieces are washed in wooden, glass or enamel tanks or under other conditions which do not produce additional deleterious influences. For example, there may be found baths which are effective in a glass tank, but which are not effective in a galvanized iron tank, or in an iron tank, when the metal being cleaned is in contact with the metal of the tank. The tank metal and the metal piece to be cleaned establish electrical contact and are in a common bath, thus establishing galvanic action. By this condition different electrical potentials between the two metals and the solution cause a galvanic flow of electricity, or alteration of the single potential which exists between each metal alone and the cleaning bath. The same conditions may occur in a non-conductive tank where different kinds of metal pieces are being cleaned in contact with each other. The alteration of conditions as a result of these galvanic couples can be sufficient to produce corrosion or injury with cleaning baths which are otherwise satisfactory.

The present invention aims to produce a detergent compound which is more universally effective for various metals to be cleaned, and for use in glass, zinc, galvanized iron, or iron tanks, and for use simultaneously with different metals to be cleaned. It is an object to provide a compound in solid form to be added to water to form a bath, or else to provide the bath itself. Although the invention provides a bath which is effective where galvanic force exists, it should be understood that the conditions which are encountered in the galvanic action are the result of forces which exist in the absence of a galvanic couple, namely the electrical potential existing between the bath and the metal to be cleaned. This potential is involved in the deleterious action to be avoided. The bath, therefore, as a

whole, creates a favorable single potential between the bath and the metal, which potential is such that it remains favorable when galvanic conditions are also encountered.

The detergent compounds in this art are generally used in concentrations varying from  $\frac{1}{2}$  to 8 ounces per gallon, and in the work leading to this invention this range of concentration has been more particularly studied. The general statements herein made are with reference to such a range of concentration, but it is not to be assumed that the general statements are not applicable above and below this range. The temperature and time of exposure to the cleaning agent also have a bearing on the action, and unless otherwise specified general statements are to be considered with reference to conditions commonly encountered in commercial practice.

Common alkaline reacting detergents are soda ash, caustic soda, trisodium phosphate, sodium silicate, borax, etc. Several of these may be used in weak solutions, such as 0.15% to 3% concentration when cold without giving corrosion, or other deleterious action, but the cleaning action is not effective. When heated to secure effective cleaning, there is also corrosion or other adverse action. Addition agents for inhibiting corrosion are recognized but they have limited or specific action depending upon concentration and kind of alkali, concentration of inhibiting agent, temperature, and time. Sodium hypochlorite is one such agent. Chromates are recognized inhibitors for mild alkaline detergents.

Calcium hypochlorite is not a successful inhibitor for use with the general run of alkaline detergent when used for tin or aluminum surfaces, and for use in glass, iron, zinc or galvanized tanks. Neither are zinc salts, such as zinc sulphate, suitable inhibitors under these conditions. The present invention is based upon the discovery that calcium hypochlorite and a zinc salt such as zinc sulphate, may be used in combination as a corrosion inhibiting mixture for alkaline detergents under the described conditions. In order best to explain the invention, typical examples of the invention are here given, and later discussed.

## Example No. 1

|                                                  | Per cent |
|--------------------------------------------------|----------|
| Trisodium phosphate monohydrate                  | 32.50 50 |
| Anhydrous sodium carbonate                       | 32.25    |
| Sodium metasilicate                              | 20.00    |
| Calcium hypochlorite (70-72% available chlorine) | 5.00 55  |
| Anhydrous zinc sulfate                           | 10.00 25 |
| Wool Orange 2-G                                  |          |

## Example No. 2

|                                  | Per cent |
|----------------------------------|----------|
| Trisodium phosphate monohydrate  | 30.00    |
| Anhydrous sodium carbonate       | 39.75    |
| 5 High test calcium hypochlorite | 6.00     |
| Anhydrous zinc sulfate           | 9.00     |
| Sodium metasilicate              | 15.00    |
| Wool Orange 2-G                  | .25      |

10

## Example No. 3

|                                 | Per cent |
|---------------------------------|----------|
| Trisodium phosphate monohydrate | 42.25    |
| Anhydrous sodium carbonate      | 42.50    |
| High test calcium hypochlorite  | 5.00     |
| 15 Anhydrous zinc sulfate       | 10.00    |
| Wool Orange 2-G                 | .25      |

10 15 15

## Example No. 4

|                                                                                    | Per cent |
|------------------------------------------------------------------------------------|----------|
| 20 Powdered borax ( $\text{Na}_2\text{B}_4\text{O}_7 \cdot 10\text{H}_2\text{O}$ ) | 24.75    |
| Sodium metasilicate                                                                | 15.00    |
| Anhydrous sodium carbonate                                                         | 45.00    |
| High test calcium hypochlorite                                                     | 5.00     |
| Anhydrous zinc sulfate                                                             | 10.00    |
| 25 Wool Orange 2-G                                                                 | .25      |

## Example No. 5

|                                 | Per cent |
|---------------------------------|----------|
| Trisodium phosphate monohydrate | 25.00    |
| Anhydrous sodium carbonate      | 39.75    |
| 30 Sodium metasilicate          | 20.00    |
| High test calcium hypochlorite  | 5.00     |
| Anhydrous zinc sulfate          | 10.00    |
| Wool Orange 2-G                 | .25      |

35 It will be observed from the above formulas that the composition is solid, being a mixture of the separate ingredients named. These are to be used in concentrations of  $\frac{1}{2}$  to 8 ounces per gallon of water. The resulting bath is not necessarily a solution of these ingredients unchanged. It must be recognized that there may be reactions between ingredients when water is present, that new compounds are formed; that even precipitates may be formed; that the solution 40 arrives at some equilibrium composition at definite conditions and is variable with change of conditions; and that in use this bath may change considerably in its composition. Precipitates may not form in making a solution, but may 45 tend to form, and they may form in use of the bath for cleaning.

The inhibiting action may be due to formation of an inhibiting film on the metal, or to the tendency to form an inhibiting film. Frequently in chemical action there is a force tending to produce a certain result. The action does not occur until a certain "threshold" value of the force is attained, yet the mere existence of the force without a visible result therefrom, is a 50 vital factor in a process.

Such a condition has been observed in studying the present invention, but there is reason to believe that it is not the only instance of such conditions. This observation relates to the 55 presence of zinc in the bath.

There have been observed certain conditions under which zinc from the solution plates out, electrochemically or galvanically, onto the metal being cleaned. This indicates that a certain 60 "threshold" value for a zinc-depositing force has been exceeded, resulting in the zinc deposition. On the low side of this limiting value for the force, the tendency for zinc to plate out must exist, yet the zinc does not deposit visibly. It 65 may be depositing invisibly at a rate equal to or

less than a rate at which it is dissolved, so that the net result is no deposition.

It is well recognized that where there is a tendency to plate onto a metal, there is little or no tendency for the metal to be dissolved by 5 the plating solution. From these facts and observations it is believed that the presence of zinc in the solution is an important factor contributing to the inhibiting action of the composition. It is quite likely that the zinc in solution 10 acts to alter the potential difference between the bath and the metal to be cleaned, from what the potential would be if the zinc were absent. However, the action of the soluble zinc appears to be joint with other ingredients. 15

## Alkaline detergent part

The invention may be practiced with the common alkaline detergents, but it is preferred that the less caustic ones be used, in order to protect 20 workers from caustic burns. Mixed alkaline detergents are preferred, and a fine mild combination consists of trisodium phosphate monohydrate, anhydrous sodium carbonate (soda ash) and sodium metasilicate ( $\text{Na}_2\text{SiO}_3 \cdot 5\text{H}_2\text{O}$ ). This 25 mixture in the present invention has the advantage of protecting iron, zinc, tin and aluminum surfaces. Borax may be substituted for the trisodium phosphate monohydrate for the protection of these metals. Where sodium metasilicate is omitted from the mixture of alkalis, the composition does not protect aluminum, but it 30 does protect the zinc, iron and tin surfaces. Example No. 3 is an example of a composition which is not effective on aluminum under the 35 regular condition of commercial usage. The alkaline detergent part of the whole composition may vary in a wide manner. In the final composition the alkaline detergent part is preferably 85% where the inhibiting part is about 15%. 40 The exact ratio is not critical and the variations may be readily determined by simple experimentation. Sodium silicate is primarily of the alkaline detergent part, but as to aluminum it also falls in the inhibiting part. There are several 45 forms of sodium silicate, and their specific effects may vary the efficiency or limiting proportions for a given set of conditions. The sodium metasilicate is preferred to others, such as sodium orthosilicate because in the dry solid composition it creates better stability. 50

## Inhibiting part

The inhibiting mixture consists of calcium hypochlorite and a zinc salt. Preferably high test 55 calcium hypochlorite and anhydrous zinc sulphate are used. These are readily powdered for admixture with the powdered alkaline detergent. Various salts of zinc may be used. Zinc sulphate is preferred to chloride or acetate. For example, 60 because the sulphate gives greater stability to the solid mixture, the examples are given in terms of sulphate. In making a bath directly the other salts may be used. The two ingredients of this part of the composition may vary in their ratio 65 to each other, and there will of course be one ratio which is more effective for a certain alkaline agent or combination of them. This efficient ratio may also vary for the conditions of use, and with variations in the ratio between the 70 alkaline part and the inhibiting part. It is therefore not possible to set forth explicitly a definite efficient ratio.

The commercially preferred ratio and form is 1 part of calcium hypochlorite (high test com- 75

mercially defined as having 70 to 72% available chlorine and containing about 3% of calcium chloride and 23% sodium chloride) and 2 parts of anhydrous zinc sulphate (about 36% zinc content). For 85% content of the preferred alkaline mixture above described, and 15% content of inhibiting part, the latter has the preferred ratio of 1 part of commercial "high test" calcium hypochlorite and 2 parts of anhydrous zinc sulphate. If this last ratio is reversed the desired effect is not obtained. The critical limit is not subject to determination unless exact specifications for use are given, and then there must be considered the extent to which the bath is allowed to deteriorate in use, before it is considered non-effective.

The important ingredient in the commercial high test calcium hypochlorite is the combination or compound of calcium, oxygen and chlorine. The sodium chloride present in the form described is not any essential part of the invention, but its presence obviously plays a part in determining critical proportions of the essential ingredients for any set of conditions. There are on the market various forms of "high test calcium hypochlorite", and in addition to the form having sodium chloride, there is a form having calcium chloride instead of sodium chloride. This may be used in the composition with appropriate adjustments, but it is not preferred where a solid powder is marketed on account of the hygroscopic nature of calcium chloride.

*The examples*

The examples show Wool Orange 2-G, but this is merely an example of a dyestuff optionally added to give character or distinction to the composition and to the bath.

Formulas Nos. 1, 2, 4 and 5 give adequate protection to iron, zinc, aluminum and tinned ware. Formula No. 3, lacking sodium silicate is adequate for iron, zinc and tinned ware, but not for aluminum ware. These formulas give such protection when the temperature is maintained above 80° C. or higher and at the boiling point for extensive periods of time longer than commercially used to effect cleaning, such as 8 hours and even to 48 hours. The effectiveness of the inhibitor may be appreciated by the fact that any of the alkaline agents alone in the same concentration (such as 85% of the 1/2 to 8 ounces per gallon) at 70° C., give corrosive action on both aluminum and tinned ware in a few minutes, and immediately at 100° C.

Formula No. 3 is exceptional in that it will deposit zinc upon tinned ware when the concentration is too high, for example over about 5 ounces per gallon. This is striking evidence of a function for zinc in the bath, at lower concentrations where it is not deposited. The tendency to deposit is no doubt an important part of the inhibiting forces.

The composition is preferred in a form which may be economically marketed. Hence ingredients are chosen which may be mixed to remain stable and non-reactive. The available chlorine from the hypochlorite may be fugitive and its retention is important. Absence of water is desirable to keep the mass stable. Steel drums are suitable containers for inducing stability in the compositions given. Although there may be water of crystallization in some of the components (particularly the borax, and the trisodium phosphate monohydrate) it is so closely bound that it is not detrimental to stability.

When the composition is dissolved reactions occur which vary with the composition and conditions. The bath may even become milky with some precipitate or insoluble suspension. Transient films may be formed on the metal to be cleaned, yet the cleaning action without deleterious action on the metal is effected. The baths may be boiled, for example for 8 hours, with little loss of available chlorine. The bath itself is stable at the commercially useful dilution.

It is to be understood that the bath itself is the functioning composition of the invention, and that it may be described as the reaction product of the constituents named in the formulas. One could make up the bath directly, and then there is more latitude in choice of ingredients. For example, sodium hypochlorite may be used in place of calcium hypochlorite. The substitution cannot readily be made in the solid powder form because sufficiently strong sodium hypochlorite is not available in solid form. The calcium form of hypochlorite is merely a means to employ hypochlorite in a strong solid form which with other ingredients produces a stable composition. The alkali emulsifies or saponifies the grease and fat and readily cleans other dirt or food residues.

The invention has several aspects as set forth herein. The formulas may be changed considerably from the examples given as indicated by the scope of the appended claims.

The present application is specific to our pending application Serial No. 220,346, filed July 20, 1938, as a continuation in part of this application with claims generic to the matter claimed herein.

We claim:

1. A corrosion-inhibiting alkaline composition for cleaning zinc, iron and tin ware in a solution thereof at from cold to boiling temperatures consisting essentially of about 85% of water soluble inorganic alkaline detergent, about 5% to 6% of a solid hypochlorite salt of a metal from the group consisting of alkali metals and alkali earth metals, and about 9% to 10% of water-soluble zinc salt.

2. A composition according to claim 1 in which the zinc salt is zinc sulphate.

3. A composition according to claim 1 in which the hypochlorite salt is calcium hypochlorite.

4. A composition according to claim 1 in which the alkaline detergent material is a mixture of anhydrous sodium carbonate and trisodium phosphate monohydrate.

5. A composition according to claim 1 which is useful in addition for aluminum ware in which part of the alkaline detergent is a sodium silicate in the amount of about 15% to 20% of the composition.

6. A corrosion-inhibiting alkaline composition for cleaning zinc, iron, tin and aluminum ware in a solution thereof at from cold to boiling temperatures consisting essentially of from about 65% to 70% of water soluble inorganic alkaline detergent, from about 15% to 20% of sodium silicate, about 5% to 6% of calcium hypochlorite, and about 9% to 10% of zinc sulphate.

7. A corrosion-inhibiting mixture for addition to a water soluble inorganic alkaline detergent to render a bath of such material non-corrosive on zinc, iron and tin ware at from cold to boiling temperatures, which consists of about 1 part of a hypochlorite salt of a metal from the group consisting of alkali metals and alkali earth met-

als, and about 2 parts of a water-soluble zinc salt.

8. The method of inhibiting the action of aqueous solutions of inorganic alkaline detergents upon zinc, iron and tin ware at temperatures from 80° C. to boiling which comprises adding to the detergent solution having about 85 parts of alkaline detergent, an inhibiting mixture consisting of about 5 to 6 parts of a hypochlorite salt of a metal from the group consisting of alkali metals and alkali earth metals, and about 9 to 10 parts of a water-soluble zinc salt.

9. The method of inhibiting the action of aqueous solutions of inorganic alkaline detergents upon zinc, iron, tin and aluminum ware at temperatures from 80° C. to boiling which comprises adding to the detergent solution having

about 65 to 70 parts of the inorganic alkaline detergent, an inhibiting mixture consisting of about 15 to 20 parts of sodium silicate, about 5 to 6 parts of a hypochlorite salt of a metal from the group consisting of alkali metals and alkali earth metals, and about 9 to 10 parts of a water-soluble zinc salt.

10. A corrosion-inhibiting mixture for addition to a water soluble inorganic alkaline detergent to render a bath of such material non-corrosive of zinc, iron and tin ware at from cold to boiling temperatures, which consists of about 1 part of a hypochlorite salt of a metal from the group consisting of alkali metals and alkali earth metals, and about 2 parts of zinc sulphate.

CARROLL L. GRIFFITH. 15  
LLOYD A. HALL.